

M. GUETT.  
METHOD OF MAKING CHARACTER PLATES.  
APPLICATION FILED APR. 14, 1920.

1,357,046.

Patented Oct. 26, 1920.

Fig. 1



Fig. 3



*M. Guett*  
Inventor  
By *Frank Sutherland*  
Attorney

# UNITED STATES PATENT OFFICE.

MONROE GUETT, OF HARTFORD, CONNECTICUT.

## METHOD OF MAKING CHARACTER-PLATES.

1,357,046.

Specification of Letters Patent. Patented Oct. 26, 1920.

Application filed April 14, 1920. Serial No. 373,846.

To all whom it may concern:

Be it known that I, MONROE GUETT, a citizen of the United States, residing at Hartford, in the county of Hartford and State of Connecticut, have invented certain new and useful Improvements in Methods of Making Character-Plates, of which the following is a specification.

This invention relates to a method of making character plates. In carrying the method into effect I use desirably as a base or foundation a piece of ferrous metal such for instance as steel or iron. This metal foundation or base piece has desirably characters usually obtained by embossing. The embossing can be secured in any convenient way. The base plate with its characters I prefer to coat with some non-ferrous metal such as nickel, copper, brass or zinc. This coating of non-ferrous material may be applied to the ferrous body in any one of several different ways, for instance by plating, hot galvanizing or otherwise. After the non-ferrous substance is applied customarily to all of the exposed surfaces of the ferrous body, being usually applied to the face thereof, the non-ferrous substance is removed from portions of the body such as from the characters in some convenient way ordinarily however by a grinding action. After the surface or surfaces have had the non-ferrous substance removed, I subject the coated article to heat treatment. This oxidizes the cleared portion or portions and makes a color or surface which appreciably and materially contrasts with that of the major part of the metal body. The ferrous metal body may function in various fashions. One of several is to put characters on it so that it will function as an index plate or dial in a rotary snap switch.

In the drawings accompanying and forming part of the present specification I have illustrated one of the several ways of carrying the procedure into effect. This will be set forth in the following description. These drawings at the same time show an article made in conformity with the method. It will be clear however that I am not restricted to the disclosure made by the drawings and description. I may in fact depart therefrom in several respects within the scope of the invention defined by the claims following said description.

55 Referring to said drawings:

Figure 1 is a face view of a plate.

Fig. 2 is a cross section on the line 2—2 of Fig. 1.

Fig. 3 is a view corresponding to Fig. 1 of a finished plate.

Fig. 4 is a cross section on the line 4—4 of Fig. 3.

Like characters refer to like parts throughout the several views which are on different scales.

In Fig. 1 I have shown a plate 2. Although this plate is shown as being in the form of a dial or disk to adapt the same for use in an electric switch, the invention as I have already noted is not restricted in this particular. The plate as shown, has on it the raised characters 3. I have also observed the fact that it may not always be necessary to raise the characters for they may be of intaglio formation. As a matter of fact the form of the plate and that of the characters thereon is an old one in electric snap switches. This plate or body 2 is of ferrous material of which steel and iron are illustrations.

The plate has desirably first applied to it a coating 4 of non-ferrous material of which I mention several. This non-ferrous material is applied to the entire exposed surface of the plate as indicated in Fig. 4. When this is done the protective coating 4 as represented is removed from the active face of the characters 3. In the case illustrated this removal would be off the topmost flat surface of said characters and the removal in question is desirably accomplished by grinding.

After the protective coating is removed from the exposed surface of the character, the article is subjected for instance about one minute to heat treatment for illustration by a furnace of some kind in which it is subjected to a temperature of approximately between 500 and 600 degrees Fahrenheit. This heat treatment oxidizes the exposed part of the plate which is the front faces of the characters 3.

As I have observed the method can be used in different fields and the article can be employed with advantage in divers connections. As to the article I have mentioned one use and have also shown the same. The plate or disk 2 has as shown the central openings 5 to receive the spindle of a snap switch.

110 What I claim is:

1. A method involving a ferrous plate

having characters thereon, comprising coating the plate with non-ferrous metal, then removing a portion of the non-ferrous coating from the ferrous plate, and finally subjecting the plate to heat treatment.

2. A method involving a ferrous plate having characters thereon, comprising coating the plate with non-ferrous metal, then removing the non-ferrous metal from the characters and finally subjecting the plate to heat treatment.

3. A method involving a ferrous plate

having characters thereon, comprising coating the plate with non-ferrous material, then removing a portion of the non-ferrous coating from the ferrous plate, and then oxidizing that part of the plate from which the non-ferrous coating has been removed.

In testimony whereof I affix my signature in the presence of two witnesses.

MONROE GUETT.

Witnesses:

A. J. BENNETT,  
MADELINE MUSSGNUG.